

[54] **TEXTILE TREATING COMPOSITIONS,  
PROCESS OF TREATING TEXTILES, AND  
TEXTILE ARTICLES**

[75] Inventor: **Barry M. Shay, Wilmington, Del.**

[73] Assignee: **ICI United States Inc., Wilmington, Del.**

[22] Filed: **June 9, 1969**

[21] Appl. No.: **831,770**

[52] **U.S. Cl.** ..... **8/187; 8/115.6; 8/115.7;  
8/DIG. 4; 8/DIG. 21; 260/29.4 R; 260/404;  
260/404.5; 260/468 L; 260/482 B; 260/482 C**

[51] **Int. Cl.** ..... **D06m 15/54; D06m 15/58**

[58] **Field of Search** ..... **8/116.3, 115.6; 260/404;  
260/404.5, 482 B, 482 C, 29.4 R**

[56] **References Cited**

**UNITED STATES PATENTS**

|           |         |                  |           |
|-----------|---------|------------------|-----------|
| 1,959,930 | 5/1934  | Schmidt et al.   | 260/404   |
| 1,970,578 | 8/1934  | Schoeller et al. | 260/404   |
| 2,002,613 | 5/1935  | Orthner et al.   | 260/404   |
| 2,157,362 | 5/1939  | Ulrich et al.    | 260/482 C |
| 2,184,008 | 12/1939 | Dickey et al.    | 260/482 C |
| 2,197,479 | 4/1940  | Meigs            | 260/482 C |
| 2,218,939 | 10/1940 | Steindorff       | 260/482 C |
| 2,477,346 | 7/1949  | Pikl             | 260/482 C |

|           |        |                |           |
|-----------|--------|----------------|-----------|
| 2,518,267 | 8/1950 | Baird et al.   | 260/404.5 |
| 2,585,826 | 2/1952 | Olsen          | 260/482 B |
| 2,998,445 | 8/1961 | Stewart et al. | 260/482 C |
| 3,427,332 | 2/1969 | Allen et al.   | 260/404.5 |
| 3,524,876 | 8/1970 | Gregson        | 8/187     |

**FOREIGN PATENTS OR APPLICATIONS**

|           |         |                |
|-----------|---------|----------------|
| 697,315   | 9/1953  | United Kingdom |
| 1,123,677 | 8/1968  | United Kingdom |
| 1,128,812 | 10/1968 | United Kingdom |
| 610,393   | 12/1960 | Canada         |

*Primary Examiner—George F. Lesmes*

*Assistant Examiner—J. Cannon*

[57] **ABSTRACT**

Disclosed are textile treating compositions comprising (1) a methylolated carbamate which is an ester of N-methylol carbamic acid or N,N-dimethylol carbamic acid and an ethylene oxide adduct of a fatty acid, fatty alcohol, fatty acid ester of a polyol, fatty amine, or fatty acid amide and (2) a durable-press agent. The textile treating compositions may be applied to textile material to improve the physical characteristics thereof; for example, durable press properties, wrinkle-resistance, tear strength, hand and abrasion resistance.

**16 Claims, No Drawings**

TEXTILE TREATING COMPOSITIONS, PROCESS  
OF TREATING TEXTILES, AND TEXTILE  
ARTICLES

This invention relates to novel textile treating compositions. More particularly, this invention relates to textile treating compositions comprising a methylolated carbamate and a durable-press agent. This invention further relates to a process of treating textile materials to improve the physical characteristics thereof, such as durable press, wrinkle resistance, tear strength, hand, and abrasion resistance, in such a way that the improvements are not destroyed by laundering, dry-cleaning, or similar operations. This invention further relates to textile materials having improved physical properties.

During the past several years, the textile industry has become involved in the durable press treatment of textile materials. The treatment is carried out by impregnating the textile material with an aqueous solution or dispersion of a textile-reactive, cross-linking, durable-press agent and then heating the impregnated material for curing. This treatment stabilizes the fibers in the configuration they had in the textile during the curing. Consequently, when a stress is applied to the treated textile and then released, the textile tends to return to the original configuration. This results in a textile material exhibiting durable press properties.

The cross-linking treatment, however, has an adverse effect on the tear strength, hand, and abrasion resistance properties of the textile material. Thus, the cross-linked textile material, although exhibiting the beneficial characteristics of durable press behavior, has poor abrasion resistance, poor hand, and poor tear strength.

It is, accordingly, an object of this invention to provide novel textile treating compositions for application to textile materials to impart thereto durable press properties, tear strength, hand, and abrasion resistance properties and which will adhere to the textile materials through numerous laundering and drycleaning cycles.

It is another object of this invention to provide a process for treating textile material in such a manner that it has durable press properties, excellent abrasion resistance, hand, and tear strength.

It is another object of this invention to provide textile materials having improved durable press properties, hand, tear strength, and abrasion resistance.

The foregoing objects and still further objects are accomplished in accordance with the present invention by providing a textile treating composition comprising a mixture or blend of a textile-reactive, cross-linking, durable-press agent and a methylolated carbamate.

The amounts of durable-press agent and methylolated carbamate present in the textile treating compositions of this invention may vary over a rather wide range and will depend somewhat on the particular durable-press agent and methylolated carbamate selected and on the particular textile material to be treated therewith. In general, the textile treating composition of this invention may contain from about 40 to 96 percent, preferably from about 55 to about 65 percent, by weight of the durable press agent and from about 60 to 4 percent, preferably from about 45 to about 35 percent, by weight of the methylolated carbamate, based on the total weight of durable press agent and methylolated carbamate.

Durable-press agents useful in the preparation of textile treating compositions in accordance with the present invention include both monomer and polymers which when applied to a textile material and cured under conditions conventional in the art undergo reaction with the textile material and impart durable press and/or wrinkle resistant characteristics to the textile material.

Durable-press agents that are preferred when practicing the present invention are the aminoplast resins. These nitrogen containing resins, when applied to textile materials and heated at temperatures from 130°C. to 200°C. in the presence of a catalyst, react with the textile material and become chemically attached thereto. Exemplary of the aminoplast resins that may be employed according to the present invention are the ethylene ureas, for example, dimethylol dihydroxy ethylene urea, dimethylol ethylene urea, ethylene urea formaldehyde, and hydroxy ethylene urea formaldehyde; urea formaldehydes, for example, propylene urea formaldehyde and dimethylol urea formaldehyde; melamine formaldehyde, for example, tetramethylol melamines, and pentamethylol melamines; carbamates, for example, alkyl carbamate formaldehydes; formaldehyde-acrolein condensation products; alkylol amides, for example, methylol formamide and methylol acetamide; acrylamides, for example, N-methylol acrylamide, N-methylol methacrylamide, and N-methylol-N-methacrylamide; diureas, for example, trimethylol acetylene diurea and tetramethylol-acetylene diurea; triazones, for example, dimethylol-N-ethyl triazone; haloacetamides; urons, for example, dimethylol uron and dihydroxy dimethylol uron. Mixtures of aminoplast resins may also be used.

Further illustrative examples of durable-press agents useful in the preparation of the textile treating compositions of this invention include aldehydes, for example, formaldehyde, glyoxyl, and  $\beta$ -hydroxy adipaldehyde; epoxides, for example, ethylene glycol diglycidyl ether and vinylcyclohexene dioxide; ethyleneimine derivatives, for example, bisaziridenylcarbonyl, and tris(1-aziridinyl) phosphine oxide; chlorohydrins; sulfone derivatives, for example, divinyl sulfone and bis(hydroxyethyl) sulfone; and sulfonium salts, for example, disodium tris( $\beta$ -sulphatoethyl) sulfonium inner salt.

Methylolated carbamates useful in the preparation of textile treating compositions in accordance with the present invention are methylolated carbamates of an ethylene oxide adduct selected from the group consisting of

1. an ethylene oxide adduct of a fatty acid containing from 12 to 28 carbon atoms,
2. an ethylene oxide adduct of a fatty alcohol containing from 12 to 28 carbon atoms,
3. an ethylene oxide adduct of a fatty amine containing from 12 to 28 carbon atoms,
4. an ethylene oxide adduct of an amide of a fatty acid containing from 12 to 28 carbon atoms,
5. an ethylene oxide adduct of an ester of a fatty acid containing from 12 to 28 carbon atoms and a polyhydric alcohol containing from 3 to 6 carbon atoms and from 2 to 6 hydroxyl groups, and
6. a partial ester of a fatty acid containing from 12 to 28 carbon atoms and an adduct of ethylene oxide and a polyhydric alcohol containing from 3 to 6 carbon atoms and from 2 to 6 hydroxyl groups.

The methylolated carbamates of this invention contain at least one oxyethylene group, at least one fatty group containing from 12 to 28 carbon atoms, and at least one



group wherein R<sub>1</sub> is hydrogen or methylol. Accordingly, the carbamates of this invention may be described as esters of N-methylol carbamic acid and N,N-dimethylol carbamic acid and the above defined ethylene oxide adducts.

The methylolated carbamates of this invention may be prepared by reacting one or more of the ethylene oxide adducts described herein with urea or with an alkyl carbamate such as ethyl or methyl carbamate and then reacting the resulting carbamate with formaldehyde. The reactions are illustrated by the following equations:



These two well-known methods of forming carbamates are described in detail in the article by Adams et al. published in Chemical Reviews, Volume 65, pages 567-602, 1965. The disclosure of this article is hereby incorporated into this application by reference. Briefly, the reaction may be carried out by heating a mixture of urea or alkyl carbamate and an ethylene oxide adduct to a temperature in the range of from about 110°C. to about 200°C. Catalysts, such as heavy metal salts of weak organic acids, zinc chloride, cobalt chloride, lead acetate, cupric acetate, boron trifluoride, aluminum isopropoxide, dibutyltin dilaurate, and dibutyltin oxide

may be used to shorten the reaction time and increase the yield. The degree of carbamylation may be controlled by varying the amounts of ethylene oxide adduct and carbamylating agent used. For example, the reaction of three mols of urea with one mol of an ethylene oxide adduct containing six hydroxyl groups will result in the formation of a carbamate containing an average of three carbamate groups. Methylol groups are then introduced by reacting the carbamate with formaldehyde, paraformaldehyde, or other convenient source of formaldehyde.

The ethylene oxide adducts which may be used to prepare the carbamates of this invention are known compounds. U.S. Pat. Nos. 1,959,930; 1,970,578; and 2,002,613, the disclosures of which are hereby incorporated hereinto by reference, disclose the preparation of ethylene oxide adducts which may be used to prepare the carbamates of this invention. Briefly, the ethylene oxide adducts may be prepared by reacting ethylene oxide with the appropriate fatty alcohol, fatty acid, fatty amine, fatty amide, or ester of fatty acid and a polyol or by reacting a fatty acid with an ether of ethylene oxide and a polyol.

Fatty alcohols which may be used to prepare the ethylene oxide adducts include saturated or unsaturated, straight or branched chain fatty alcohols having from 12 to 28 carbon atoms. A preferred group of fatty alcohols may be represented by the formula ROH wherein R is an alkyl group or an alkenyl group containing from 12 to 28 carbon atoms. Illustrative examples of such fatty alcohols include dodecanol, dodecenol, tetradecanol, tetradecenol, hexadecanol, hexadecenol, octadecanol, octadecenol, eicosanol, eicosenol, docosanol, docosenol, tetracosanol, tetracosenol, hexacosanol, hexacosenol, octacosanol, and octacosenol.

Fatty acids which may be used to prepare the ethylene oxide adducts include saturated and unsaturated fatty acids having from 12 to 28 carbon atoms. A preferred group of fatty acids may be represented by the formula ROH wherein R is an acyl group containing from 12 to 28 carbon atoms. Illustrative examples of such fatty acids include lauric acid, myristic acid, palmitic acid, margaric acid, stearic acid, oleic acid, arachidic acid, behenic acid, lignoceric acid, cerotic acid, lauroleic acid, myristoleic acid, palmitoleic acid, oleic acid, linolenic acid, ricinoleic acid, eicosenoic acid, docosenoic acid, and tetracosenoic acid.

Fatty amines which may be used to prepare the ethylene oxide adducts include primary or secondary, saturated or unsaturated amines containing at least one fatty group having from 12 to 28 carbon atoms. A preferred group of fatty amines may be represented by the formula R'R'NH wherein R is an alkyl or alkenyl group containing from 12 to 28 carbon atoms and R' is hydrogen or an alkyl or alkenyl group containing from 1 to 28 carbon atoms. Illustrative examples of such fatty amines include dodecylamine, hexadecylamine, octadecylamine, eicosylamine, pentacosylamine, didodecylamine, dioctadecylamine, N-methyldodecylamine, N-ethyloctadecylamine, ARMEEN TD, ARMEED SD cocoamine, oleyl amine.

Fatty amides which may be used to prepare the ethylene oxide adducts include fatty amides having at least one fatty group containing from 12 to 28 carbon atoms. A preferred group of fatty amides may be represented by the formula RNR'H wherein R is an acyl group containing from 12 to 28 carbon atoms and R' is hydrogen

or an alkyl or alkenyl group containing from 1 to 28 carbon atoms. Illustrative examples of such fatty amides include dodecanamide, hexadecanamide, octadecanamide, octadecenamide, eicosanamide, pentacosanamide, N-methyl-octadecanamide, N-stearyl-hydroxystearamide, dodecanamide, N-oleyl-octadecanamide, N-oleyl-pentadecenamide, and N-lauryl-stearamide.

Polyols which may be used to prepare the ethylene oxide adducts include polyols having from 3 to 6 carbon atoms and from 2 to 6 hydroxyl groups. A preferred group of polyols may be represented by the formula  $R(OH)_m$  wherein R is an aliphatic group having from 3 to 6 carbon atoms and m is from 2 to 6. Illustrative examples of these polyols include propylene glycol, hexamethylene glycol, butanediol, isosorbide, isomannide, glycerine, hexanetriol, pentaerythritol, erythritol, sorbitan, mannitan, sorbitol, mannitol, dulcitol, querцитol, inositol, and arabitol.

The methylolated carbamates of this invention may be characterized by a formula selected from the group consisting of the following generalized formulae wherein identical symbols have identical signification:



2.  $R_3(OA)_x$ ,



and

4.  $(R_5O)_yD$

wherein

R is an alkyl group containing from 12 to 28 carbon atoms, an alkenyl group containing from 12 to 28 carbon atoms, an acyl group containing from 12 to 28 carbon atoms, or the group resulting from removing a hydroxyl group from lanolin,

$R_1$  is hydrogen or  $-CH_2OH$ ,

n is an integer from 1 to 150,

$R_3$  is the group remaining after removing all the hydroxyl groups from a saturated, aliphatic alcohol having from 3 to 6 carbon atoms and from 2 to 6 hydroxyl groups,

x is an integer from 2 to 6,

each

A is independently selected from the group consisting of hydrogen, alkyl groups containing from 12 to 28 carbon atoms, alkenyl groups containing from 12 to 28 carbon atoms, acyl groups containing from 12 to 28 carbon atoms,



and  $+CH_2 - CH_2 - O +_n R_6$  wherein  $R_6$  is hydrogen, an acyl group containing from 12 to 28 carbon atoms, or



with the proviso that at least one A contains an alkyl, alkenyl, or acyl group containing from 12 to 28 carbon atoms, at least one A contains a  $+CH_2 - CH_2 - O +_n R_6$  group, and at least one A contains



group,

$R_4$  is an alkyl group containing from 12 to 28 carbon atoms, an alkenyl group containing from 12 to 28 carbon atoms, or an acyl group containing from 12 to 28 carbon atoms,

each

B is independently selected from the group consisting of alkyl groups containing from 1 to 28 carbon atoms, alkenyl groups containing from 1 to 28 carbon atoms, and  $+CH_2 - CH_2 - O +_n R_{10}$  wherein  $R_{10}$  is hydrogen or



35 with the proviso that at least one B contains a



group,  $R_5$  is H or



45 with the proviso that at least one  $R_5$  is



55 y is a number from 1 to 5, and

D is the group remaining after removing all the hydroxyl groups from an adduct of ethylene oxide and an ester of a fatty acid having from 12 to 28 carbon atoms and a polyol having from 2 to 6 hydroxyl groups and from 3 to 6 carbon atoms.

In order that those skilled in the art may better understand the nature and preparation of the methylolated carbamates, the following examples are given. These examples are set forth solely for the purpose of illustration and any specific enumeration of details con-

tained therein should not be interpreted as expressing limitations of this invention. All parts and percentages are by weight, unless otherwise stated.

The following procedure is employed in Examples 1 to 27. The indicated amounts of urea and ethylene oxide adduct are charged to a three-necked flask and the contents of the flask heated to the indicated temperature for the indicated length of time. The reaction product is filtered to remove any unreacted urea. The filtrate is the carbamate of the starting ethylene oxide adduct. The recovered carbamate is then mixed with a 37 percent aqueous solution of formaldehyde and heated to about 50°C. for 10 to 12 hours to form the methylolated carbamate.

5

using other durable press agents and methylolated carbamates for those recited. The textile treating composition of Example 32 is a preferred embodiment of this invention.

## EXAMPLE 32

|                                    |     |
|------------------------------------|-----|
| Carbamate of Example 24            | 40% |
| Dimethylol dihydroxy ethylene urea | 60% |

## EXAMPLE 33

|                                         |     |
|-----------------------------------------|-----|
| Carbamate of Example 1                  | 45% |
| 1,3-Dimethylol hexahydro-pyrimidinone-2 | 55% |

10

15

| Example Number | Ethylene Oxide Adduct                              | Grams of Adduct | Grams of Urea | Temperature °C. | Time-Hours | Carbamate <sup>(1)</sup> Hydroxy | Methylol <sup>(2)</sup> Carbamate |
|----------------|----------------------------------------------------|-----------------|---------------|-----------------|------------|----------------------------------|-----------------------------------|
| 1              | Polyoxyethylene(4) lauryl alcohol                  | 200             | 35.6          | 155             | 13         | 0.67                             | 1.2                               |
| 2              | Dioleate of polyoxyethylene(20)sorbitol            | 60              | 5.8           | 150             | 9          | 0.62                             | 1.2                               |
| 3              | Polyoxyethylene(15)castor oil                      | 500             | 5.8           | 160             | 6          | 0.66                             | 1.2                               |
| 4              | Polyoxyethylene(20)tall oil                        | 200             | 13.4          | 160             | 9          | 0.6                              | 1.2                               |
| 5              | Polyoxyethylene(20)ether of glycerol dioleate      | 106             | 5.3           | 150-160         | 5½         | 0.69                             | 1.2                               |
| 6              | Polyoxyethylene(20)ether of lanolin                | 200             | 7.8           | 160             | 7          | 0.27                             | 1.2                               |
| 7              | Polyoxyethylene(20)ether of glycerol monopalmitate | 200             |               | 155-160         | 7½         | 0.83                             | 1.2                               |
| 8              | Polyoxyethylene(40)-N-stearyl-12-hydroxystearamide | 200             | 3.5           | 160             | 6%         | 0.42                             | 1.2                               |
| 9              | Polyoxyethylene(20)ether of sorbitan monooleate    | 200             | 17            | 155-160         | 6¼         | 0.64                             | 1.2                               |
| 10             | Polyoxyethylene(30)stearic acid                    | 200             | 10.4          | 160             | 4          | 0.51                             | 1.2                               |
| 11             | Polyoxyethylene(5)ARMBEN DS                        | 100             | 26            | 155-165         | 6¼         | 0.83                             | 1.2                               |
| 12             | Polyoxyethylene(14)cocoamine                       | 100             | 16.6          | 150             | 5¾         | 1                                | 1.2                               |
| 13             | Polyoxyethylene(20)sorbitan monolaurate            | 100             | 33            | 150             | 7          | 1                                | 1.2                               |
| 14             | Polyoxyethylene(20)sorbitan monostearate           | 100             | 27.6          | 150             | 5          | 0.95                             | 1.2                               |
| 15             | Dioleate of polyoxyethylene(20)sorbitol            | 100             | 15            | 150             | 7          | 9.8                              | 1.2                               |
| 16             | Polyoxyethylene(5)octadecylamine                   | 100             | 24            | 150-160         | 12         | 0.6                              | 1.2                               |
| 17             | Polyoxyethylene(20)ARMEEN TD                       | 100             | 19.8          | 155             | 6          | 0.6                              | 1.2                               |
| 18             | Polyoxyethylene(25)hydrogenated castor oil         | 100             | 8.4           | 155             | 6          | 0.5                              | 1.2                               |
| 19             | Polyoxyethylene(54)castor oil                      | 100             | 6.6           | 155             | 7¼         | 0.9                              | 1.2                               |
| 20             | Polyoxyethylene(81)castor oil                      | 100             | 4.5           | 150-165         | 10         | 0.6                              | 1.2                               |
| 21             | Polyoxyethylene(150)hydrogenated castor oil        | 100             | 3.2           | 155             | 6¾         | 0.75                             | 1.2                               |
| 22             | Polyoxyethylene(50)octadecylamine                  | 100             | 6             | 150             | 12         | 0.77                             | 1.2                               |
| 23             | Dioleate of polyoxyethylene(3)sorbitol             | 100             | 24            | 170-175         | 6½         | 0.8                              | 1.2                               |
| 24             | Polyoxyethylene(25)hydrogenated castor oil         | 100             | 5.6           | 155             | 7          | 0.53                             | 1.7                               |
| 25             | Polyoxyethylene(25)hydrogenated castor oil         | 100             | 10.1          | 155             | 7          | 1                                | 1.5                               |
| 26             | Polyoxyethylene(25)hydrogenated castor oil         | 600             | 100.1         | 155             | 6¾         | —                                | 1                                 |
| 27             | Polyoxyethylene(25)hydrogenated castor oil         | 600             | 33.2          | 155             | 7          | —                                | 1.6                               |

<sup>(1)</sup>Number of carbamate groups introduced per hydroxy group in ethylene oxide adduct charged (by analysis for non-urea nitrogen).

<sup>(2)</sup>Number of N-methylol groups per carbamate group.

The procedure of Examples 1 to 27 is followed in Examples 28 to 31 except that the indicated amount of ethyl carbamate is used instead of urea and a toluene aze trope is used to remove the liberated ethanol. 100 grams of the indicated ethylene oxide adduct are employed in each example.

45

50

## EXAMPLE 34

|                                     |     |
|-------------------------------------|-----|
| Carbamate of Example 8              | 35% |
| Dimethylol-5-hydroxy propylene urea | 65% |

| Example Number | Ethylene Oxide Adduct                      | Grams of Ethyl-Carbamate | Temperature °C. | Time-Hours | Carbamate <sup>(1)</sup> Hydroxy | Methylol <sup>(2)</sup> Carbamate |
|----------------|--------------------------------------------|--------------------------|-----------------|------------|----------------------------------|-----------------------------------|
| 28             | Polyoxyethylene(5)octadecylamine           | 44.5                     | 140             | 9¾         | 0.8                              | 1.2                               |
| 29             | Polyoxyethylene(25)hydrogenated castor oil | 13.3                     | 130             | 6          | 0.9                              | 1.2                               |
| 30             | Polyoxyethylene(20)sorbitan monolaurate    | 48.5                     | 130             | 10¾        | 1                                | 1.2                               |
| 31             | Polyoxyethylene(5)octadecylamine           | 44.5                     | 135             | 12½        | 0.8                              | 1.2                               |

<sup>(1)</sup>Number of carbamate groups introduced per hydroxy group in ethylene oxide adduct charged.

<sup>(2)</sup>Number of N-methylol groups per carbamate group.

The following are illustrative examples of the textile treating compositions of this invention. All percentages are by weight. It is understood, of course, that additional textile treating compositions may be prepared by

65

## EXAMPLE 35

|                                        |     |
|----------------------------------------|-----|
| Methylolated carbamate of Example 2    | 60% |
| Dimethylol-5,5-dimethyl propylene urea | 40% |

## EXAMPLE 36

Methyloated carbamate of Example 10  
Dimethylol methoxy ethyl carbamate

4%  
96%

5

## EXAMPLE 37

Methyloated carbamate of Example 26  
Methyloated carbamate of Example 9  
Dimethylol dihydroxy ethylene urea

20%  
20%  
60%

## EXAMPLE 38

Methyloated carbamate of Example 16  
Disodium tris ( $\beta$ -sulphatoethyl) sulfonium  
inner salt  
Dimethylol hexahydropyrimidinone-2

42%  
38%  
20%

In accordance with the present invention, the above described textile treating compositions containing a durable press agent and a methyloated carbamate may be used to treat textile materials to impart thereto improved physical characteristics such as durable press, wrinkle resistance, tear strength, hand, and abrasion resistance. It has been found that if the textile treating compositions of this invention are applied to textile material along with a textile resin catalyst and the treated textile material heated to an elevated temperature, the durable press agent and the methyloated carbamate will be attached to the textile material so that the improved properties imparted to the textile material will not be removed by subsequent washing or drycleaning.

The textile resin catalyst may be any of the acid or latent acid catalysts which are conventionally used in the art to facilitate reaction of durable press agents with textile material. By latent acid catalysts is meant substances which develop acidity during the curing step. Particularly suitable catalyst include metal salts of strong acids such as magnesium chloride, magnesium sulfate, and zinc nitrate; ammonium salts such as ammonium chloride and ammonium dihydrogen phosphate; amine salts such as triethylamine hydrochloride, and triethanolamine hydrochloride. The amount of curing catalyst used will depend on the nature of the durable agent, the particular carbamate used, and on the curing temperature and curing time. In general, satisfactory results may be obtained by using from about 5 percent to about 40 percent, preferably from about 10 percent to about 25 percent by weight of the catalyst based on the total weight of durable press agent and methyloated carbamate.

The textile treating compositions of this invention may be applied to textile materials from an aqueous medium. The pad bath may contain a surfactant or emulsifier. Illustrative examples of surfactants which may be used include polyoxyethylene(12)tridecyl alcohol, polyoxyethylene(9)octylphenol, and polyoxyethylene(9.2)nonyl phenol.

The textile materials may be treated with the bath containing the textile treating compositions of this invention by immersion therein or by spraying. In the immersion method of application, the textile material may either be run through a padding machine wherein the textile material is first dipped into the bath and then squeezed, or the textile materials may be dipped into

the bath and the excess liquid extracted by centrifugation. In the spraying method of application, the textile materials are simply sprayed with the bath and then dried by any suitable means. The carbamate and durable press agent may be applied simultaneously or from separate baths. The catalyst for the durable press agent may be applied with the durable press agent and/or carbamate or from a separate bath.

The amount of a textile treating compositions of this invention which is applied to the textile material may vary from about 1 percent to about 20 percent, preferably from about 4% to about 10%, by weight based on the dry weight of the textile material.

It is necessary to subject the textile material having a textile treating composition of this invention thereon to an elevated temperature in order to initiate a curing reaction between the said composition and the textile material. The particular temperature used and the duration of the heating step depends on the nature of the textile material used and on the the particular methyloated carbamate and durable-press resin used. In each situation, however, the temperature and heating time is that necessary to sufficiently cause reaction of the methyloated carbamate and durable-press resin with the textile material. Generally, the heat cure may be effective at temperatures from about 100°F. to about 350°F. and in periods of time ranging from about 40 to 60 minutes at the lower temperature to about 2 to 3 minutes at the higher temperature. The preferred temperature is from about 300°—350°F.

Textile materials which may be treated with the textile compositions of this invention include any textile material containing active hydrogen atoms; for example, textile material comprising cellulose or modified cellulose such as cotton, rayon, linen, and mixtures thereof; textile material containing noncellulosics such as nylon, acrylics, polyesters, and mixtures thereof; and textile materials comprising a blend of cellulosic materials and non-cellulosic materials. The textile materials may be in the form of filaments, fibers, threads and yarns or in the form of woven, nonwoven, knit, or otherwise formed fabrics, sheets, and cloths. The preferred textile material is woven cotton fabric and cotton/polyester blends.

The following examples are illustrative of the application of textile treating compositions of this invention to textile materials. The physical properties of the treated textile materials are determined according to the following test procedures.

45 Monsanto crease angle recovery — ASTM D1295-60T

Elmendorf tear strength — ASTM D1424-59

Stoll-Flex abrasion resistance — ASTM D1175-61T

55 In examples 39 to 52, scoured swatches of Testfabric's Style No. 413 bleached, mercerized cotton twill are padded at 70 percent wet pickup on the Butterworth Pad with an aqueous bath containing 3.6 percent of the indicated carbamate, 5.4 percent of dimethylol dihydroxy ethylene urea durable-press agent, 1.2 percent of zinc nitrate catalyst, and 0.25% of polyoxyethylene (9.2) nonyl phenol wetting agent. The bath is prepared by mixing the carbamate with the durable-press agent, adding the wetting agent, diluting with warm water, and adding an aqueous solution of the catalyst. The padded fabrics are dried 5 minutes at 225°F., cured at 325°F. for 10 minutes, and conditioned at 70°F. and 65 percent R. H. for sixteen hours. Half of

the swatches from each treatment are washed ten times in an automatic washing machine with TIDE and hot water. The properties of the treated fabrics are shown in Table I.

TABLE I

| Example Number | Carbamate of Example | Monsanto Crease Angle Recovery W+F (Degrees) |           | Elmendorf Warpwise Tear Strength (lb.) |           | Stoll-Flex Abrasion Resistance (W+F) (cycles) |           |
|----------------|----------------------|----------------------------------------------|-----------|----------------------------------------|-----------|-----------------------------------------------|-----------|
|                |                      | 0 Wash                                       | 10 Washes | 0 Wash                                 | 10 Washes | 0 Wash                                        | 10 Washes |
| 39             | 3                    | 282                                          | 264       | 2.6                                    | 2.4       | 1423                                          | 1385      |
| 40             | 1                    | 247                                          | 232       | 2.4                                    | 1.8       | 1744                                          | 1111      |
| 41             | 4                    | 243                                          | 249       | 2.1                                    | 1.5       | 1956                                          | 1231      |
| 42             | 5                    | 257                                          | 246       | 2.3                                    | 1.6       | 1262                                          | 1446      |
| 43             | 6                    | 260                                          | 242       | 2.0                                    | 1.8       | 1162                                          | 1289      |
| 44             | 7                    | 271                                          | 247       | 2.2                                    | 1.7       | 1393                                          | 929       |
| 45             | 8                    | 258                                          | 239       | 2.3                                    | 1.6       | 906                                           | 1045      |
| 46             | 9                    | 267                                          | 239       | 2.2                                    | 1.4       | 1152                                          | 912       |
| 47             | 10                   | 260                                          | 239       | 2.2                                    | 1.3       | 1097                                          | 1983      |
| 48             | 11                   | 228                                          | 232       | 2.8                                    | 3.2       | 1636                                          | 1813      |
| 49             | 12                   | 238                                          | 236       | 2.0                                    | 2.2       | 1244                                          | 1579      |
| 50             | 30                   | 246                                          | 252       | 1.7                                    | 1.6       | 1085                                          | 1148      |
| 51             | 13                   | 256                                          | 257       | 2.1                                    | 1.8       | 1039                                          | 891       |
| 52             | 14                   | 268                                          | 245       | 2.5                                    | 2.2       | 1473                                          | 1409      |

In Examples 53 to 56, swatches of cotton poplin fabric are padded at 70% wet pickup on the Butterworth Pad with an aqueous bath containing 4.95% dimethylol dihydroxy ethylene urea, 4% of the indicated carbamate, 1.4% of zinc nitrate, and 0.25% of polyoxyethylene (9.2) nonyl phenol. The treated fabrics are dried for 5 minutes at 210°F., cured at 325°F. for 10 minutes, and conditioned at 70°F. and 65% R. H. for twelve hours. The properties of the treated fabrics, prior to washing and after 10 washings, are shown in Table II.

TABLE II

worth Pad with an aqueous bath containing 1% of the methylolated carbamate of Example 24, 9 percent of dimethylol dihydroxy ethylene urea, 1.4 percent of zinc nitrate, and 0.25 percent of polyoxyethylene (9.2) nonyl phenol. The padded fabrics are dried for five minutes at 210°F. and cured for ten minutes at 325°F. The treated fabric has a Monsanto Crease Angle Recovery in the warp plus fill directions of 298° prior to washing and 274° after ten washings, a Stoll-Flex abrasion resistance in the warp plus fill directions of 689 cy-

| Example Number | Carbamate of Example | Monsanto Crease Angle Recovery W+F (Degrees) |           | Elmendorf Warpwise Tear Strength (lb.) |           | Stoll-Flex Abrasion Resistance (W+F) (cycles) |           |
|----------------|----------------------|----------------------------------------------|-----------|----------------------------------------|-----------|-----------------------------------------------|-----------|
|                |                      | 0 Wash                                       | 10 Washes | 0 Wash                                 | 10 Washes | 0 Wash                                        | 10 Washes |
| 53             | 18                   | 290                                          | 262       | 1.31                                   | 1.39      | 1039                                          | 954       |
| 54             | 19                   | 281                                          | 255       | 1.24                                   | 0.99      | 1033                                          | 840       |
| 55             | 20                   | 276                                          | 248       | 1.16                                   | 1.04      | 966                                           | 723       |
| 56             | 21                   | 282                                          | 255       | 1.23                                   | 1.04      | 974                                           | 700       |

In Examples 57 and 58, scoured swatches of Testfabric's Style No. 7402M fabric comprising a blend of 65 percent DACRON S4 polyester and 35% cotton poplin are padded at 57 percent wet pickup on the Butterworth Pad with an aqueous bath containing 6.2 percent dimethylol dihydroxy ethylene urea, 5.1 percent of the indicated carbamate, 1.7 percent of zinc nitrate, and 0.25% of polyoxyethylene (9.2) nonyl phenol. The padded fabric swatches are dried at 200°F. for three minutes, cured at 325°F. for 10 minutes, and conditioned at 70°F. and 65 percent R. H. for twelve hours. The physical characteristics of the swatches, prior to washing and after ten washings in hot TIDE solution, are shown in Table III.

cles prior to washing and 584 cycles after ten washings, and an Elmendorf tear strength in the warp direction of 1.27 pounds prior to washing and 1.34 pounds after ten washings. The treated fabric has a subjective hand rating of 2.2 prior to washing and 2.2 after ten washings. The subjective hand rating is a measure of softness, and the numerical rating increases as the softness decreases. Cotton fabric treated in accordance with the above described process, except that the pad bath does not contain the methylolated carbamate, shows a subjective hand rating of 3.8 prior to washing and 3.2 after ten washings.

It will be understood that the compositions of the present invention as described herein and defined in

TABLE III

| Example Number | Carbamate of Example | Monsanto Crease Angle Recovery W+F (Degrees) |           | Elmendorf Warpwise Tear Strength (lb.) |           | Stoll-Flex Abrasion Resistance Warp Only (cycles) |           |
|----------------|----------------------|----------------------------------------------|-----------|----------------------------------------|-----------|---------------------------------------------------|-----------|
|                |                      | 0 Wash                                       | 10 Washes | 0 Wash                                 | 10 Washes | 0 Wash                                            | 10 Washes |
| 57             | 26                   | 307                                          | 310       | 6.15                                   | 4.23      | 873                                               |           |
| 58             | 27                   | 312                                          | 311       | 6.12                                   | 4.40      | 943                                               |           |

the claims include those compositions containing the named ingredients and any other ingredients which do not destroy the effectiveness of the compositions for the purpose stated in the specification and, although this invention has been described with reference to specific reactant materials, including specific methylolated carbamates, ethylene oxide adducts, methylolating agents, and catalysts, it will be apparent that still other different and equivalent materials may be substituted for those described. Moreover, application processes and reaction steps thereof may be modified, reversed, or even in some cases eliminated, all within the spirit and scope of this invention.

Having described the invention, what is desired to be secured by Letters Patent is:

1. A textile treating composition comprising a durable press agent and an N-methylol or N,N-dimethylol carbamate of an ethylene oxide adduct selected from the group consisting of (1) an ethylene oxide adduct of a fatty acid containing from 12 to 28 carbon atoms, (2) an ethylene oxide adduct of a secondary fatty amine containing from 12 to 28 carbon atoms, (3) an ethylene oxide adduct of an ester of a fatty acid having from 12 to 8 carbon atoms and a polyol having from 2 to 6 hydroxyl groups and from 3 to 6 carbon atoms, and (4) a partial ester of a fatty acid having from 12 to 28 carbon atoms and an oxyethylene adduct of a polyol having from 2 to 6 hydroxyl groups and from 3 to 6 carbon atoms.

2. A textile treating composition of claim 1 wherein the carbamate is a carbamate of an ethylene oxide adduct of a fatty acid containing from 12 to 28 carbon atoms.

3. A textile treating composition of claim 1 wherein the carbamate is a carbamate of an ethylene oxide adduct of a secondary fatty amine containing from 12 to 28 carbon atoms.

4. A textile treating composition of claim 1 wherein the carbamate is a carbamate of an ethylene oxide adduct of an ester of a fatty acid having from 12 to 28 carbon atoms and a polyol having from 2 to 6 hydroxyl groups and from 3 to 6 carbon atoms.

5. A textile treating composition of claim 4 wherein the ester is castor oil.

6. A textile treating composition of claim 4 wherein the ester is hydrogenated castor oil.

7. A textile treating composition of claim 4 wherein the ethylene oxide adduct is polyoxyethylene (25) hydrogenated castor oil.

8. A textile treating composition of claim 1 wherein

20

25

30

35

40

45

50

the carbamate is a carbamate of a partial ester of a fatty acid having from 12 to 28 carbon atoms and an oxyethylene adduct of a polyol having from 2 to 6 hydroxyl groups and from 3 to 6 carbon atoms.

9. A textile treating composition of claim 8 wherein the fatty acid is oleic acid and the polyol is sorbitol.

10. A textile treating composition comprising dimethylol dihydroxy ethylene urea and an N-methylol or N,N-dimethylol carbamate of an ethylene oxide adduct selected from the group consisting of

1. an ethylene oxide adduct of a fatty acid containing from 12 to 28 carbon atoms,

2. an ethylene oxide adduct of a fatty alcohol containing from 12 to 28 carbon atoms,

3. an ethylene oxide adduct of a fatty amine containing from 12 to 28 carbon atoms,

4. an ethylene oxide adduct of an ester of a fatty acid containing from 12 to 28 carbon atoms and a polyhydric alcohol containing from 3 to 6 carbon atoms and from 2 to 6 hydroxyl groups, and

5. a partial ester of a fatty acid containing from 12 to 28 carbon atoms and an adduct of ethylene oxide and a polyhydric alcohol containing from 3 to 6 carbon atoms and from 2 to 6 hydroxyl groups.

11. A textile treating composition of claim 10 wherein the carbamate is a carbamate of an ethylene oxide adduct of a fatty alcohol containing from 12 to 28 carbon atoms.

12. A textile treating composition of claim 10 wherein the carbamate is a carbamate of an ethylene oxide adduct of a fatty amine containing from 12 to 28 carbon atoms.

13. A process of treating textile material containing cotton which comprises applying to the textile material, a textile treating composition of claim 1 and an acidic curing catalyst and thereafter curing by heating the textile material to an elevated temperature.

14. A process of treating textile material containing cotton which comprises applying to the textile material, a textile treating composition of claim 10 and an acidic textile resin curing catalyst and thereafter curing by heating the textile material to an elevated temperature.

15. An article of manufacture which comprises a textile material treated in accordance with the process of claim 13.

16. An article of manufacture which comprises a textile material treated in accordance with the process of claim 14.

\* \* \* \* \*

UNITED STATES PATENT AND TRADEMARK OFFICE  
CERTIFICATE OF CORRECTION

PATENT NO. : 3,897,208  
DATED : July 29, 1975  
INVENTOR(S) : Barry M. Shay

It is certified that error appears in the above-identified patent and that said Letters Patent are hereby corrected as shown below:

Column 4, line 30, "exmaples" should read -- examples --.

Column 4, line 61, "ARMEED" should read -- ARMEEN --.

Column 6, line 48, "Ch<sub>2</sub>OH" should read -- CH<sub>2</sub>OH --.

Column 7, Example 11, "ARMBEN" should read -- ARMEEN --.

Column 8, Example 15, "9.8" should read -- 0.8 --.

Column 8, lines 18 & 54, "Carbamate<sup>(1)</sup>" should read -- Carbamate<sup>(1)</sup> / --.  
Hydroxy Hydroxy

Column 8, lines 18 & 54, "Methylol<sup>(2)</sup>" should read -- Methylol<sup>(2)</sup> / --.  
Carbamate Carbamate

Column 13, line 24, "to 8 carbon" should read -- to 28 carbon --.

Signed and Sealed this  
*Thirteenth Day of September 1977*

[SEAL]

Attest:

RUTH C. MASON  
Attesting Officer

LUTRELLE F. PARKER  
Acting Commissioner of Patents and Trademarks